

July 22, 1958

W. A. WESLEY ET AL

2,844,530

BLACK NICKEL PLATING

Filed Feb. 15, 1957



INVENTORS  
Waclaw Andrew Wesley  
By Burton Bower Knapp  
C. A. Weller  
ATTORNEY

1

2,844,530

## BLACK NICKEL PLATING

Waclaw Andrew Wesley, Plainfield, and Burton Bower Knapp, Westfield, N. J., assignors to The International Nickel Company, Inc., New York, N. Y., a corporation of Delaware

Application February 15, 1957, Serial No. 640,373

15 Claims. (Cl. 204—40)

The present invention relates to a novel bath composition and process for producing decorative surfaces on metallic articles and, more particularly, to a novel electroplating bath solution and process for the electrodeposition of black nickel finishes on metallic surfaces and to the production of articles of manufacture having black nickel finishes.

It is well known that metal articles having lustrous black finishes are desirable and suitable for numerous applications and uses, particularly for decorative purposes and/or to promote absorption or radiation of heat. Too, matte black finishes are important in providing non-reflecting surfaces in industrial and military instruments of various types, the protoscope being an example of the former, the naval anemometer an example of the latter. However, black nickel deposits produced heretofore have been found unsatisfactory in various applications because of poor abrasion resistance and/or poor adherence of the nickel deposit to the metallic surfaces and/or poor ductility characteristics. Moreover, prior art black nickel plating processes, in addition to yielding films characterized by unsatisfactory physical properties, have been found difficult to control so as to produce a uniform black nickel coating. It has been recognized that factors contributing to difficulties encountered in the "controllability" of known black nickel plating processes often stem from the comparatively rigid and restrictive operating conditions imposed by such processes, particularly anent pH control, range of concentration of the constituents of the plating baths, current density limits, plating times, etc. For example, the normal operating range for the pH of the well-known sulfate-type plating baths, which are perhaps the baths most commonly used in commercial practice, generally falls within the relatively narrow range of about 5 to 6. When the pH of such baths falls below about 5, the nickel deposits often become undesirably dull and unattractive and, as a consequence thereof, careful regulation and control of pH values is required. In addition thereto, the concentrations of various constituents commonly employed in sulfate-type solutions must be controlled within rather narrow limits. Too, the permissible current densities employed in many sulfate-type plating baths are often of a narrow and restrictive scope, e. g., about 0.5 to about 1.5 amperes per square foot. It will be appreciated that such rather severe restrictions with respect to operating conditions

2

manifest the practical necessity for a commercial black nickel plating process and electroplating solution which provide flexibility in operating procedure and facility of control while providing a black nickel finish having improved physical properties. Although many attempts were made to overcome the foregoing difficulties and other difficulties, none, as far as we are aware, was entirely successful when carried into practice commercially on an industrial scale.

10 It has now been discovered that a decorative, black finish may be applied uniformly and without difficulty to metallic surfaces by employing a special electrolytic bath composition and process to produce a black nickel electro-deposit which is uniform in color and exhibits an improved combination of properties with respect to abrasion resistance, adhesivity and ductility.

It is an object of the present invention to provide decorative colored surfaces on metallic articles.

20 Another object of the invention is to provide a durable, substantially permanent black color on metallic surfaces for decorative purposes, to prevent reflection of light and/or to promote absorption or radiation of heat.

25 The invention also contemplates providing metallic surfaces with electrodeposited black finishes characterized by strong adhesivity, good ductility, and substantial resistance to abrasion.

30 It is also the purpose of the invention to provide nickel and/or nickel-coated materials with uniform and substantially permanent black nickel finishes which exhibit a superior combination of physical properties as compared to black nickel finishes heretofore known.

35 It is a further object of the invention to provide a novel electrolytic solution for producing tough, permanent, jet black finishes on metallic surfaces.

40 The invention further contemplates providing a novel electroplating bath for depositing a decorative jet black color on nickel and/or nickel-coated materials.

It is another object of the invention to provide a novel 45 electroplating bath for the provision of ductile, adherent and abrasion-resistant black nickel finishes on metallic surfaces, particularly nickel and/or nickel-coated materials.

Still another object of the invention is to provide a 50 novel aqueous electroplating bath of special composition for the provision of uniform black nickel finishes on metallic surfaces which is conducive to ease of control and facility of operation in the electrodeposition of such black nickel finishes.

55 It is also an object of the invention to provide a novel process for accomplishing the foregoing objects.

It is likewise within the contemplation of the instant 60 invention to provide a process for blackening metallic articles which is easily controllable and provides uniform coatings.

Among the further objects of the present invention is the provision of articles of manufacture with decorative black finishes characterized by an improved combination of properties with respect to abrasion resistance, ductility and adhesion.

Other objects and advantages will become apparent from the following description taken in conjunction with the accompanying drawing which sets forth a graph depicting the relationship between current density and nickel chloride hexahydrate concentration in the special plating bath contemplated in accordance with the invention.

Generally speaking, the present invention contemplates the electrodeposition of durable black nickel finishes upon metallic articles, particularly nickel and nickel-coated articles, by subjecting the metallic articles to the action of an aqueous, acidic electroplating bath containing nickel chloride hexahydrate, ammonium chloride, sodium thiocyanate and zinc chloride, the nickel chloride hexahydrate concentration and current density being related such that the correlation falls within the shaded area ABCDA of the accompanying graph. The black nickel finishes produced in accordance with the concepts of the instant invention are characterized by a highly satisfactory combination of physical properties, including abrasion resistance, ductility, and adhesivity of the black nickel deposit to the metallic surface treated. Moreover, as shown by the graph, nickel chloride hexahydrate-current density relationships falling outside the shaded area of the graph result in inferior black nickel deposits. For example, a nickel chloride hexahydrate-current density relationship above the shaded area results in irregular, grey deposits; a relationship falling below the shaded area results in dark grey deposits.

The constituents of our electroplating solution can be varied over relatively wide range of concentration and this factor is an extremely important commercial consideration because it advantageously assists in minimizing the prior difficulties encountered in controlling black nickel plating processes. The concentrations of the respective components of our aqueous plating bath are maintained as follows: nickel chloride ( $\text{NiCl}_2 \cdot 6\text{H}_2\text{O}$ ), at least about 50 g. p. l. (grams per liter), e. g., 50 to about 165 g. p. l.; ammonium chloride ( $\text{NH}_4\text{Cl}$ ), about 7.5 to about 45 g. p. l.; sodium thiocyanate ( $\text{NaCNS}$ ), about 7.5 g. p. l. to about 30 g. p. l.; and zinc chloride ( $\text{ZnCl}_2$ ), about 15 to about 60 g. p. l. Preferably, the bath contains about 60 to about 90 g. p. l. of nickel chloride hexahydrate, about 15 to about 30 g. p. l. of ammonium chloride, about 10 to about 20 g. p. l. of sodium thiocyanate, and about 20 to about 50 g. p. l. of zinc chloride. We have found that it is important within the principles of the instant invention that the concentrations of ammonium chloride and zinc chloride not fall below a minimum of about 7.5 g. p. l. and approximately 15 g. p. l., respectively. Amounts of ammonium chloride below about 7.5 g. p. l. produce unattractive, rough grey deposits. Likewise, when the minimum amount of zinc chloride falls below about 15 g. p. l., an undesirable light grey color results.

One of the attendant advantages and features of the present invention is that uniform black finishes are obtained with a minimum amount of regulation and control during the electrodeposition operation. Not only does our plating bath permit of an appreciable latitude in varying the concentrations of the respective constituents but the pH, current density and plating time may also be varied over comparatively wide ranges. With respect to pH, the data set forth in Table I hereinbelow illustrates that the pH can be varied over the relatively wide range of from at least as low as pH 2.3 to at least about pH 5.5. The electroplating solution of the present invention containing nickel chloride hexahydrate, ammonium chloride, sodium thiocyanate and zinc chloride generally has a pH value of the order of 5 to about 5.5. If it is desired to operate at lower pH values, the pH can be readily adjusted by adding to the bath a small amount of acid, preferably hydrochloric acid in an amount up to about 0.5 milliliter per liter of electroplating solution. An equivalent amount of sulfuric acid can be used but is less preferred.

|                                           |                 |    |
|-------------------------------------------|-----------------|----|
| Black nickel plating solution:            |                 |    |
| $\text{NiCl}_2 \cdot 6\text{H}_2\text{O}$ | g. p. l.        | 75 |
| $\text{NH}_4\text{Cl}$                    | g. p. l.        | 30 |
| $\text{NaCNS}$                            | g. p. l.        | 15 |
| $\text{ZnCl}_2$                           | g. p. l.        | 30 |
| Plating conditions:                       |                 |    |
| Temperature                               | room.           |    |
| Cathode                                   | wrought nickel. |    |
| Anode                                     | wrought nickel. |    |

| Run No. | pH  | Current Density, a. s. f. | Time, Minutes | Cathode Appearance |
|---------|-----|---------------------------|---------------|--------------------|
| 1       | 5.5 | 1.5                       | 30            | Good Black Color.  |
| 2       | 5.0 | 1.5                       | 30            | Do.                |
| 3       | 4.6 | 1.5                       | 30            | Do.                |
| 4       | 4.2 | 1.5                       | 30            | Do.                |

<sup>1</sup>pH obtained by adding hydrochloric acid.

The above variation in pH values did not alter the appearance of the electrodeposited black nickel films in any manner and it will be readily appreciated that obviating the necessity of close pH control and regulation is decidedly advantageous and particularly beneficial in providing an easily controllable process.

Another advantage of the present invention is that substantially thick black nickel deposits can be obtained if desired under a given set of operating conditions since the electrodeposition process can be conducted for relatively long periods of time without deleteriously affecting the attractive black appearance of the electrodeposited film. Generally, there is normally a minimum time interval required to produce a black film at a particular current density. Plating periods below this minimum value usually result in dark films having some color interference. When the plating period is allowed to continue for relatively long periods of time beyond the minimum time interval, a thicker film develops but it remains black in color. This factor permits the build-up of thick black deposits on the metallic surface being treated and by so doing it serves a two-fold purpose. First, careful regulation of the plating period above a minimum time interval is substantially obviated and secondly, the thick deposits so obtained materially assist in providing good abrasion resistance. Table II hereinbelow sets forth by way of illustration various plating periods that may be suitably employed for current densities of 1.5 a. s. f. and higher.

Table II

|                                           |             |               |
|-------------------------------------------|-------------|---------------|
| Black nickel plating solution:            |             | as indicated. |
| $\text{NiCl}_2 \cdot 6\text{H}_2\text{O}$ | 30 g. p. l. |               |
| $\text{NH}_4\text{Cl}$                    | 15 g. p. l. |               |
| $\text{NaCNS}$                            | 30 g. p. l. |               |

|                     |                 |  |
|---------------------|-----------------|--|
| Plating conditions: |                 |  |
| Temperature         | room.           |  |
| Cathode             | wrought nickel. |  |

| Run No. | pH  | Current Density, a. s. f. | Time, Minutes | $\text{NiCl}_2 \cdot 6\text{H}_2\text{O}$ , g. p. l. | Cathode Appearance                           |
|---------|-----|---------------------------|---------------|------------------------------------------------------|----------------------------------------------|
| 5       | 5.3 | 1.5                       | 7.5           | 75                                                   | Good Dark Color But Some Interference Color. |
| 6       | 5.3 | 1.5                       | 15            | 75                                                   | Good Dark Black.                             |
| 7       | 5.3 | 1.5                       | 30            | 75                                                   | Do.                                          |
| 8       | 5.5 | 1.5                       | 15            | 75                                                   | Do.                                          |
| 9       | 5.5 | 1.5                       | 30            | 75                                                   | Do.                                          |
| 10      | 5.2 | 1.5                       | 30            | 60                                                   | Do.                                          |
| 11      | 5.2 | 3.0                       | 15            | 105                                                  | Do.                                          |
| 12      | 5.2 | 3.0                       | 30            | 105                                                  | Do.                                          |
| 13      | 5.1 | 3.0                       | 30            | 105                                                  | Do.                                          |
| 14      | 5.1 | 6.0                       | 7.5           | 150                                                  | Do.                                          |
| 15      | 5.1 | 6.0                       | 30            | 150                                                  | Do.                                          |

<sup>1</sup>Nickel-plated steel cathode.

In run 5 a dark color was obtained having some interference color. The plating time was 7.5 minutes indicating that a borderline time had elapsed for the deposition of a good dark black color. When the plating time was increased to 15 minutes as shown by run 6, a good dark black finish was obtained. In run 7, the development of

a good black film of increasing thickness was still continuing after a plating period of 30 minutes. If short plating periods will serve the intended purpose or are required by economical and commercial considerations, plating intervals at least as low as 7.5 minutes can be satisfactorily employed in accordance with the present invention since the current density can be increased to at least about 6 a. s. f. This feature is illustrated by run 14 of Table II. Again, a thicker deposit could be obtained by extending the plating period of run 14, for example, to 30 minutes as shown in run 15 of Table II.

We have also discovered that the abrasion resistance and adhesion of black nickel finishes can be further improved by subjecting the surface of the material to be blackened to a pre-treatment operation wherein an initial or preliminary metal electrodeposit, preferably nickel, is applied to the surface prior to the aforescribed black plating treatment. It has been found that when the pre-treatment operation is employed, black finishes are obtained having a markedly improved combination of superior abrasion resistance and adhesion as compared to black finishes heretofore known. It is preferred to provide the initial nickel electrodeposit from an acid-nickel chloride bath containing not more than about 350 g. p. l. of nickel chloride hexahydrate, the pH of the bath being not more than pH 3. Preferably, the pre-treating bath contains up to about 35 g. p. l. of boric acid, up to about 40 g. p. l. of hydrochloric acid and about 150 to about 340 g. p. l. of nickel chloride hexahydrate.

A preferred acid-nickel chloride pre-treatment operation comprises immersing the article to be treated in an aqueous bath solution containing about 150 to about 240 g. p. l. of nickel chloride hexahydrate and about 30 to about 40 g. p. l. of hydrochloric acid. The bath is maintained at a temperature of about 60° F. to about 80° F. at a pH of about 0 to about 0.5. The article to be plated is treated anodically for about 1 to about 3 minutes and then cathodically for about 5 to about 10 minutes while employing suitable current densities of about 20 to about 40 a. s. f.

Of course, other pre-treatment operations can be satisfactorily employed to provide the preliminary nickel electrodeposit. For example, a nickel electrodeposit from a pre-treating bath containing about 30 g. p. l. of boric acid and about 300 g. p. l. of  $\text{NiCl}_2 \cdot 6\text{H}_2\text{O}$  has given excellent results. The operating conditions for this bath were as follows: temperature, 140° F.; pH, about 2; and current density, about 50 a. s. f. A small amount of anti-pitting agent, about 0.2 g. p. l., sold as Duponol ME, was added to the bath.

The data tabulated in Table III is illustrative of the combination of excellent adhesion and abrasion properties obtained when using the acid-nickel chloride pre-treatment process and affords a comparison of results when wrought nickel and nickel-plated steel panels were subjected to known conventional pre-treating processes as well as to the acid-nickel chloride pre-treatment process. The acid-nickel chloride treatment involved treating the materials in an aqueous bath maintained at about 75° F. and containing about 180 g. p. l. of nickel chloride ( $\text{NiCl}_2 \cdot 6\text{H}_2\text{O}$ ) and approximately 36 g. p. l. of hydrochloric acid. An electric current was passed therethrough at a current density of about 30 a. s. f. and the articles were treated anodically for approximately 2 minutes and then cathodically for about 6 minutes. The panels were rinsed in clean water and then subjected to the action of our plating bath under conditions set forth in Table III herein. Each panel was then tested for both abrasion resistance and adhesivity. The abrasion test consisted of revolving a pencil eraser in contact with the surface of the respective panels at about 625 revolutions per minute with sufficient pressure to deform the eraser. The test was conducted for periods of 1, 3, 5, 10 and 20 seconds on different portions of the panels. With respect to the adhesion test, all runs were conducted by subjecting each panel to a severe bend test wherein a free bend

was applied through an angle of 180° which gave a bend with a radius of about  $\frac{1}{16}$  inch to  $\frac{1}{4}$  inch.

Table III

|    |                                           |                 |    |  |  |  |
|----|-------------------------------------------|-----------------|----|--|--|--|
| 5  | Black nickel plating solution:            |                 |    |  |  |  |
|    | $\text{NiCl}_2 \cdot 6\text{H}_2\text{O}$ | g. p. l.        | 75 |  |  |  |
|    | $\text{NH}_4\text{Cl}$                    | g. p. l.        | 30 |  |  |  |
|    | $\text{NaCNS}$                            | g. p. l.        | 15 |  |  |  |
|    | $\text{ZnCl}_2$                           | g. p. l.        | 30 |  |  |  |
| 10 | Plating conditions:                       |                 |    |  |  |  |
|    | Temperature                               | room.           |    |  |  |  |
|    | Anode                                     | wrought nickel. |    |  |  |  |
|    | pH                                        | 5.5             |    |  |  |  |
|    | Current density                           | 1.5 a. s. f.    |    |  |  |  |
|    | Time                                      | 30 minutes      |    |  |  |  |

| Run No. | Cathode Material    | Pre-treatment <sup>1</sup> | Abrasion Test, <sup>2</sup> Seconds |   |   |    |    | Adhesion Bend Test |
|---------|---------------------|----------------------------|-------------------------------------|---|---|----|----|--------------------|
|         |                     |                            | 1                                   | 3 | 5 | 10 | 20 |                    |
| 15      | Wrought Nickel      | P                          |                                     |   | E | G  | F  | Poor.              |
| 16      | do                  | PCS                        |                                     |   | E | G  | F  | Fairly.            |
| 17      | do                  | PCH                        |                                     |   | E | G  | F  | Good.              |
| 20      | do                  | PCA                        |                                     |   |   |    | E  | Very.              |
| 18      | do                  | PCH                        |                                     |   | E | G  | F  | Poor.              |
| 19      | do                  | PCA                        |                                     |   |   |    | E  | Excellent.         |
| 20      | Nickel-Plated Steel | None                       | E                                   | G | F | F  | F  | Very.              |
| 21      | do                  | OS                         |                                     |   | E | G  | F  | Poor.              |
| 25      | do                  | CH                         |                                     |   | E | G  | F  | Fairly.            |
| 22      | do                  | CA                         |                                     |   |   |    | E  | Good.              |
| 23      | do                  | CA                         |                                     |   |   |    | E  | Fair.              |
|         |                     |                            |                                     |   |   |    |    | Excellent.         |

<sup>1</sup> P—pumice scrub; C—cathodic alkaline clean; S—25%  $\text{H}_2\text{SO}_4$  dip; H—15% (vol.)  $\text{HCl}$  dip; A—Acid-nickel chloride treatment.

<sup>2</sup> E, G, F and P represent the rating of excellent, good, fair and poor, respectively.

It will be noted that in only runs Nos. 19 and 23 was a rating of excellent (E) obtained for both abrasion resistance (20 second periods) and adhesivity and in each of these experiments the material being plated was subjected to the acid-nickel chloride pre-treatment process described hereinbefore. Although a severe bending test was applied for determining the adhesive qualities of the respective finishes, there was no indication of chipping, peeling, flaking, etc., of the black coating formed in accordance with our invention and using our aforescribed pre-treatment process. The data concerning the bend test of 180° also serves to illustrate that the black finishes produced in accordance with our invention, while utilizing the preferred pre-treatment process (runs Nos. 19 and 23), are highly ductile.

Metals other than nickel which can be satisfactorily used as the preliminary metal electrodeposit include copper, silver, cobalt, chromium, lead, cadmium, zinc, tin, antimony, bismuth and gold. Alloys such as cobalt-nickel, tin-bismuth, antimony-bismuth and brass can also be suitably employed as preliminary metal electrodeposits.

For many purposes, black matte finishes are also desired. In such instances the material to be plated is given a matte surface by mechanical, chemical or other means. However, black matte finishes provided on such surfaces heretofore have exhibited the undesirable effect of lacking adhesivity. In accordance with the present invention, black matte finishes are easily achieved and the finish is strongly adherent.

The present invention can be employed to provide black finishes on a wide variety of foundation metals and/or alloys such as stainless steel, steel, copper alloys, cast iron, precious metals, and alloys thereof, etc., and is particularly applicable for producing black decorative coatings on nickel and/or nickel-coated materials, e. g., wrought nickel, electrodeposited nickel. The instant invention is suitable for such applications as nickel-plated steel, baking pans, office machines, name plates, jewelry, photographic equipment, etc.

It will be apparent from the foregoing that the instant invention provides a novel aqueous electrolytic bath and an electrodeposition process which is easily controllable in providing jet black finishes on metallic surfaces,

Since concentrations of nickel chloride, ammonium chloride, sodium thiocyanate, and zinc chloride may be suitably varied over relatively wide ranges and since a wide latitude is permitted in variations of pH values, current densities and plating times, careful control and regulation of the process is substantially minimized. It will be readily apparent that the flexibility in operating conditions of the instant invention provides the art with a process which may be conveniently adapted to fulfill a particular need or requirement. For example, if an attractive black-finish is desired in a minimum time interval, a suitably high current density, e. g., 6 or 7 a. s. f., may be satisfactorily employed. If a thick black deposit is desired, the plating operation can be conducted for substantially long periods of time. Moreover, the present invention is adaptable for providing matte black finishes as well as lustrous black finishes. Furthermore, when the preferred acid nickel chloride pre-treatment process is employed in conjunction with the plating operation, a superior combination of improved properties with respect to abrasion resistance and adhesion is obtained.

The term "nickel chloride hexahydrate" has been used herein to define the content of nickel chloride in the black plating solution for convenience in expression since, as those skilled in the art will readily appreciate, the nickel chloride is usually added as nickel chloride hexahydrate but the content of nickel chloride in the solution can be provided by any suitable means.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A bath for electrodepositing substantially permanent black, decorative finishes on nickel-surfaced materials and comprising an aqueous solution having a pH within a range of at least as low as about 2.3 and up to about 5.5 and containing about 60 g. p. l. to about 90 g. p. l. of nickel chloride hexahydrate, about 15 g. p. l. to about 30 g. p. l. of ammonium chloride, about 10 g. p. l. to about 20 g. p. l. of sodium thiocyanate and about 20 g. p. l. to about 50 g. p. l. of zinc chloride.

2. A bath for electrodepositing black finishes on metallic surfaces and comprising an aqueous, acidic solution containing about 50 g. p. l. to about 165 g. p. l. of nickel chloride hexahydrate, from 7.5 g. p. l. to about 45 g. p. l. of ammonium chloride, about 7.5 g. p. l. to about 30 g. p. l. of sodium thiocyanate and from 15 g. p. l. to about 60 g. p. l. of zinc chloride.

3. A bath for electrodepositing black finishes on metallic articles and comprising an aqueous, acidic solution containing at least about 50 g. p. l. of nickel chloride hexahydrate, from 7.5 g. p. l. to about 45 g. p. l. of ammonium chloride, about 7.5 g. p. l. to about 30 g. p. l. of sodium thiocyanate and from 15 g. p. l. to about 60 g. p. l. of zinc chloride.

4. A process for electrodepositing attractive black finishes on metallic articles which comprises subjecting the article to be blackened to the action of an aqueous electroplating solution having a pH within a range of at least as low as about 2.3 and up to about 5.5 and containing from 7.5 g. p. l. to about 45 g. p. l. of ammonium chloride, about 7.5 g. p. l. to about 30 g. p. l. of sodium thiocyanate, from 15 g. p. l. to about 60 g. p. l. of zinc chloride, and nickel chloride hexahydrate, the nickel chloride hexahydrate concentration and current density being related such that the correlation falls within the shaded area ABCDA of the accompanying graph.

5. A method as described in claim 4 wherein the metal to be blackened has a nickel surface.

6. An easily controllable process for electrodepositing substantially permanent and uniform black, decorative finishes on metallic articles which comprises subjecting the article to be blackened to the action of an aqueous electroplating solution having a pH within a range of at least as low as about 2.3 up to about 5.5 and containing about 15 g. p. l. to about 30 g. p. l. of ammonium chloride, about 10 g. p. l. to about 20 g. p. l. of sodium thiocyanate, about 20 g. p. l. to about 50 g. p. l. of zinc chloride, and nickel chloride hexahydrate, the concentration of said nickel chloride hexahydrate being related to the current density employed such that the correlation thereof falls within the shaded area ABCDA of the accompanying graph.

7. A method as described in claim 6 wherein the metal to be blackened is nickel-surfaced.

8. A process for providing durable, uniform and attractive black finishes on metallic articles which comprises the steps of pre-treating the article to be blackened by providing an initial metal electrodeposit thereon and then subjecting the pre-treated article to the action of an aqueous electroplating solution having a pH within a range of at least as low as about 2.3 up to about 5.5 and containing from 7.5 g. p. l. to about 45 g. p. l. of ammonium chloride, about 7.5 g. p. l. to about 30 g. p. l. of sodium thiocyanate, from 15 g. p. l. to about 60 g. p. l. of zinc chloride, and nickel chloride hexahydrate, the concentration of said nickel chloride hexahydrate being related to the current density employed such that the correlation thereof falls within the shaded area ABCDA of the accompanying graph.

9. A method as described in claim 8 wherein the initial metal electrodeposit is nickel.

10. A method as described in claim 9 wherein the metal to be blackened is nickel-surfaced.

11. An easily controllable process for providing durable, uniform and attractive black finishes on metallic articles which comprises the steps of pre-treating the article to be blackened by providing an initial metal electrodeposit thereon and then subjecting the pre-treated article to the action of an aqueous electroplating solution having a pH within a range of at least as low as about 2.3 and up to about 5.5 and containing from 15 g. p. l. to 30 g. p. l. of ammonium chloride, about 10 g. p. l. to about 20 g. p. l. of sodium thiocyanate, from 20 g. p. l. to 50 g. p. l. of zinc chloride, and nickel chloride hexahydrate, the concentration of said nickel chloride hexahydrate being related to current density such that the correlation thereof falls within the shaded area ABCDA of the accompanying graph.

12. A method as described in claim 11 wherein the initial metal electrodeposit is nickel.

13. An easily controllable process for electrodepositing durable and uniform, black attractive finishes on metallic articles which comprises the steps of immersing the metallic article in an acid-nickel chloride electrolyte containing acid and not more than about 350 g. p. l. of nickel chloride hexahydrate, the pH of the electrolyte being not more than about pH 3 to thereby provide the said metallic article with an initial electrodeposit of nickel, and then subjecting the metallic article so treated to the action of an aqueous electroplating solution having a pH within a range of at least as low as about 2.3 and up to 5.5 and containing from 7.5 g. p. l. to about 45 g. p. l. of ammonium chloride, about 7.5 g. p. l. to about 30 g. p. l. of sodium thiocyanate and from 15 g. p. l. to about 60 g. p. l. zinc chloride, and nickel chloride hexahydrate, the concentration of said nickel chloride hexahydrate being related to the current density employed such that the correlation thereof falls within the shaded area ABCDA of the accompanying graph.

14. A process as described in claim 13 wherein the

said acid-nickel chloride electrolyte contains up to 35 g. p. l. of boric acid, up to about 40 g. p. l. of hydrochloric acid and about 150 g. p. l. to about 340 g. p. l. of nickel chloride hexahydrate.

15. A process as described in claim 14 wherein the 5 said acid-nickel chloride electrolyte contains about 150 to about 240 g. p. l. of nickel chloride hexahydrate and about 30 to 40 g. p. l. of hydrochloric acid and the article is treated in said electrolyte anodically for about 1

to 3 minutes and then cathodically for about 5 to 10 minutes and the current is passed through the said electrolyte at a current density of about 20 a. s. f. to about 40 a. s. f.

References Cited in the file of this patent

UNITED STATES PATENTS

2,679,475 Singler ----- May 25, 1954

UNITED STATES PATENT OFFICE  
CERTIFICATE OF CORRECTION

July 22, 1958

Patent No. 2,844,530

Waclaw Andrew Wesley et al.

It is hereby certified that error appears in the printed specification of the above numbered patent requiring correction and that the said Letters Patent should read as corrected below.

Column 3, line 36, for "(NiCl<sub>2</sub>.6H<sub>2</sub>O)," read -- (NiCl<sub>2</sub>.6H<sub>2</sub>O), --; column 4, line 50, Table II, under the heading "Black nickel plating solution:", second formula, for "NH<sub>4</sub>Cl" read -- NH<sub>4</sub>Cl --; column 5, line 60, for "(NiCl<sub>2</sub>.6H<sub>2</sub>O)" read -- (NiCl<sub>2</sub>.6H<sub>2</sub>O) --.

Signed and sealed this 16th day of December 1958.

(SEAL)

Attest:

KARL H. AXLINE  
Attesting Officer

ROBERT C. WATSON  
Commissioner of Patents